

# United States Patent [19]

Tachibana et al.

[11] 3,906,425

[45] Sept. 16, 1975

[54] **OXIDE SEMICONDUCTOR-METAL CONTACT RESISTANCE ELEMENTS**

[75] Inventors: **Kan-Ichi Tachibana; Michihiro Nishioka; Mikiya Ono**, all of Kitakyusku, Japan

[73] Assignee: **Mitsubishi Mining & Cement Company, Ltd.**, Tokyo, Japan

[22] Filed: **May 21, 1973**

[21] Appl. No.: **362,461**

[30] **Foreign Application Priority Data**

June 22, 1972 Japan..... 47-62588

[52] U.S. Cl. .... **338/20**

[51] Int. Cl. .... **H01c 7/10**

[58] **Field of Search** ..... 338/13, 20, 22, 25; 252/512-513, 518-520; 317/234 N, 238, 235 K, 235 Q; 357/28, 57

[56] **References Cited**

UNITED STATES PATENTS

2,027,277 1/1936 Habann..... 338/20

|           |         |                    |           |
|-----------|---------|--------------------|-----------|
| 2,590,894 | 4/1952  | Sanborn.....       | 338/20    |
| 3,105,800 | 10/1963 | Watanabe.....      | 338/22 SD |
| 3,310,766 | 3/1967  | Downong et al..... | 338/20    |
| 3,393,448 | 7/1968  | Harget et al.....  | 338/22 R  |
| 3,511,786 | 5/1970  | Brixner.....       | 338/25 X  |

*Primary Examiner*—C. L. Albritton

*Attorney, Agent, or Firm*—Edward J. Brenner

[57]

## ABSTRACT

New oxide semiconductor-metal contact resistance elements having remarkably stable volt-ampere characteristics are provided. The contact resistance elements comprise oxide semiconductors which have negative resistance and also possess such thermister constant  $B^{\circ}\text{K}$  and specific resistance  $R_o\text{K}\Omega$  at  $273^{\circ}\text{K}$  as satisfy the relation  $B \times R_o \leq 10^4\text{K}\Omega^{\circ}\text{K}$ , and metals which are highly anticorrosive and have high electric conductivity, attached thereto, and are based on utilization of the property of the contact surfaces between the oxide semiconductors and the metals.

1 Claim, 4 Drawing Figures



FIG. 1.



FIG. 2.



FIG. 3.



FIG. 4.



## OXIDE SEMICONDUCTOR-METAL CONTACT RESISTANCE ELEMENTS

### BACKGROUND OF THE INVENTION

This invention relates to oxide semiconductor-metal contact resistance elements comprising oxide semiconductors and metals or alloys attached thereto. The contact resistance elements of this invention have the same remarkably stable volt-ampere characteristics as those of non-linear resistors, and these volt-ampere characteristics are based on the property of the contact surfaces between the oxide sintered bodies and the metals or alloys, consequently the contact resistance elements can be made to be small-sized.

Conventional non-linear resistors (the term "non-linear resistor" is hereinafter referred to as "varistor") comprise silicon carbide varistors, silicon varistors, barium titanate varistors and the like.

In general, the volt-ampere characteristic of such a varistor is given by the following equation (1):

$$I = I_0 \left( \frac{V}{V_0} \right)^\alpha \quad (1)$$

where  $I$  is the current flowing through the varistor,  $V$  is the voltage across the varistor,  $V_0$  is the voltage applied to the opposite surfaces of the varistor at  $I=I_0mA$ , that is, a threshold voltage, and  $\alpha$ , an index representing non-linearity is usually 3~5.

Silicon carbide varistors become worse in characteristics with smaller in size, then exhibiting  $\alpha$  values less than 3. Silicon varistors and barium titanate varistors are both able to be small-sized, but are limited in uses because  $V_0$  values thereof are as low as 0.5~1.2V.

This invention has been devised to overcome the defects of the conventional non-linear resistors as described hereinabove.

### SUMMARY OF THE INVENTION

A primary object of this invention is to provide a non-linear resistor which has a remarkably stable volt-ampere characteristic.

Another object of this invention is to provide a non-linear resistor which is able to be small-sized.

A further object of this invention is to provide a non-linear resistor which is inexpensive in cost.

According to this invention, there is provided an oxide semiconductor-metal contact resistance element comprising an oxide semiconductor, said oxide semiconductor having negative resistance and also possessing the thermister constant  $B^\circ K$  and the specific resistance value  $R_0 K\Omega$  at  $273^\circ K$  that satisfy the relation  $B \times R_0 \leq 10,000 K\Omega^\circ K$ , and a metal, said metal being highly anti-corrosive and having high electric conductivity, attached thereto.

In general, the relation between the resistance  $R K\Omega$  at  $T^\circ K$ ,  $R_0 K\Omega$  and  $B^\circ K$  of an oxide semiconductor is given by the following equation (2):

$$R = R_0 \exp \left[ B \left( \frac{1}{T} - \frac{1}{273} \right) \right] \quad (2)$$

The equation (2) is not always applicable to any temperature range, but this invention relates to  $R_0$  and  $B$  in the temperature range which the equation (2) is applicable to.

The contact resistance element of this invention is characterized in that it has an excellent characteristic which does not be lowered when made to be smaller-sized. Namely, the contact resistance element of this invention has a remarkably stable characteristic because  $V_0$  value thereof is  $10\sim20 V$  at  $I_0=5mA$  and also  $\alpha$  is about 5, and can be easily made to be smaller-sized.

The invention is now explained in detail with reference to the attached drawings.

### BRIEF DESCRIPTION OF THE ATTACHED DRAWINGS

FIG. 1 is a plan view of a preferred embodiment of this invention.

FIG. 2 shows a section view thereof.

FIG. 3 shows a volt-ampere characteristic suitable for a non-linear resistor.

FIG. 4 shows a volt-ampere characteristic unsuitable for a non-linear resistor.

20 In FIG. 3 and FIG. 4, voltage  $E$  is plotted as abscissa and current  $I$  as ordinate.

### DETAILED DESCRIPTION OF THE INVENTION

The oxide semiconductors as one component of the contact resistance element of this invention which have negative resistance and also possess such a specific resistance  $R_0 K\Omega$  at  $273^\circ K$  and a thermister constant  $B^\circ K$  that satisfy the relation  $B \times R_0 \leq 10^4 K\Omega^\circ K$  are preferably sintered bodies of the mixtures such as iron oxide and copper oxide, cobalt oxide and nickel oxide, iron oxide and titanium oxide and the rest, and the metals or alloys as another component thereof which are highly anti-corrosive and have high electric conductivity are preferably such metals as copper, zinc, nickel etc., or such alloys as brass, phosphor bronze, German silver etc. Therefore, the components of the contact resistance element of this invention are both inexpensive in cost.

Now, the contact resistance element of this invention is explained with reference to the attached drawings.

FIG. 1 shows a plan view of a preferred embodiment of this invention. FIG. 2 is a section view thereof.

The invention provides a contact resistance element, as shown in FIG. 1 and FIG. 2, manufactured easily by making small holes in the oxide sintered body 1, attaching the metal or alloy pieces 2, 2 to the oxide sintered body 1 through the small holes and fixing the whole with a suitable insulating coating material 3 such as epoxy resin. The contact resistance element of this invention has such a remarkably stable volt-ampere characteristic as shown in FIG. 3, proving to be suitable for a non-linear resistor.

55 This invention, as described hereinabove, provides a contact resistance element which is inexpensive in both raw material cost and manufacturing cost and can be made to be small-sized without lowering the remarkably stable characteristic thereof, consequently it is industrially of great value.

The invention will be understood more readily with reference to the following example. However, the example is intended to illustrate the invention and is not to be construed to limit the scope of the invention.

### EXAMPLE

The sintered body is prepared by a conventional technique. The starting material in the composition defined in Table 1 is respectively mixed in a pot mill so

as to produce a homogeneous mixture. The mixture is dried in a dryer, pressed in a mold at a pressure of about 1,000kg/cm<sup>2</sup> into a disc of 10mm in diameter and 1mm in thickness. The molded disc is sintered in air at above 1,000°C, thus the sintered disc 1 is obtained.

A contact resistance element is manufactured, as shown in FIG. 1, by making two small holes of about 1mm in diameter in the sintered disc 1, attaching the copper pieces 2, 2 to the sintered disc 1 through the two small holes respectively and fixing the whole with 10 epoxy resin 3.

As the thus manufactured contact resistance element has a surface barrier existing at the contacting surface between the sintered disc 1 and the copper piece 2 as described hereinabove, the resistance  $R_1$  thereof is high at the low voltage and the current varies as the voltage increases as shown in FIG. 3. The measured values of  $R_1$ ,  $R_0$  and  $\alpha$  of the contact resistance element are shown in Table 1. Further, the values of the resistance  $R_0$ KΩ and thermister constant  $B^\circ K$  of the sintered body 15 measured in a conventional manner are also shown in Table 1, together with those of  $R_0 \times B$ .

Table 1

| Sample No.                            | I     | II    | III   | IV    |
|---------------------------------------|-------|-------|-------|-------|
| Fe <sub>2</sub> O <sub>3</sub> (mol%) | 66    | 50    | 40    | 34    |
| CuO (mol%)                            | 34    | 50    | 60    | 66    |
| $R_0$ (KΩ)                            | 0.5   | 0.1   | 0.04  | 0.01  |
| $B$ ( $^\circ K$ )                    | 2,100 | 1,900 | 1,100 | 1,500 |
| $R_1$ (KΩ)                            | 20    | 19    | 17    | 16    |
| $V_0$ (V)                             | 19    | 18    | 16    | 15    |
| $\alpha$ (—)                          | 5     | 5     | 4     | 4     |
| $R_0 \times B$ (KΩ· $^\circ K$ )      | 1,050 | 190   | 44    | 15    |

As Table 1 shows, the values of  $R_0 \times B$  of the sintered bodies 1~IV are all not more than 10,000KΩ· $^\circ K$ . The contact resistance elements manufactured, as shown in FIG. 1, by using these sintered bodies show all the remarkably stable volt-ampere characteristics as shown

in FIG. 3, thus proving to be suitable for a non-linear resistor.

For comparison, the sintered bodies are prepared in the same manner as the above mentioned example 5 from the starting materials in the composition defined in Table 3. The measured values of  $R_0$ ,  $B$  and  $R_1$  are also shown in Table 2.

Table 2

| Sample No.                            | V      | VI     | VII    | VIII   |
|---------------------------------------|--------|--------|--------|--------|
| Fe <sub>2</sub> O <sub>3</sub> (mol%) | 70     | 0      | 0      | 50     |
| MnO <sub>2</sub> (mol%)               | 0      | 70     | 66     | 0      |
| CoO (mol%)                            | 30     | 30     | 34     | 50     |
| $R_0$ (KΩ)                            | 20     | 20     | 10     | 6      |
| $B$ ( $^\circ K$ )                    | 4,500  | 4,500  | 6,000  | 3,500  |
| $R_1$ (KΩ)                            | 140    | 140    | 30     | 25     |
| $R_0 \times B$ (KΩ· $^\circ K$ )      | 90,000 | 90,000 | 60,000 | 21,000 |

As Table 2 shows, the values of  $R_0 \times B$  of the sintered bodies V~VIII are all larger than 10,000Ω· $^\circ K$ . The contact resistance elements manufactured by attaching the copper pieces to the sintered bodies in the same manner as the above mentioned example show all the unstable volt-ampere characteristics as shown in FIG. 4, thus proving to be unsuitable for a non-linear resistor.

What is claimed is:

1. An oxide semiconductor-metal contact resistance element comprising a disk-like oxide semiconductor having a surface barrier resistance, said oxide semiconductor having negative resistance and also possessing a specific resistance value  $R_0$ KΩ at 273°K and a thermister constant  $B^\circ K$  that satisfy the relation  $R_0 \times B \leq 10,000K\Omega \cdot K$ , and two pieces of metal brought in direct and fixed contact therewith respectively, said metal being highly anticorrosive and having high electric conductivity.

\* \* \* \* \*